

Dec. 4, 1962

L. DAVIS, JR

3,067,140

ORIENTATION OF FERRITES

Filed June 16, 1959



FIG. 1



FIG. 2



FIG. 3

INVENTOR  
LUTHER DAVIS, JR.  
BY *H. Vincent Faraha*  
ATTORNEY

1

3,967,140

## 5,507,196 ORIENTATION OF FERRITES

**Luther Davis, Jr., Wayland, Mass., assignor to Raytheon Company, Lexington, Mass., a corporation of Delaware**

, Lexington, Mass., a corporation of Massachusetts.  
Filed June 16, 1958. Ser. No. 820,783.

14 Claims. (Cl. 252—62.5)

This invention relates generally to ferromagnetic, ferroelectric, and ferrite materials, and more particularly to a method of orienting the particles of these materials into a predetermined fixed disposition, and to the resulting structures attained. For the purposes of this application, the slight difference which technically exists between ferromagnetic and ferrimagnetic materials is to be disregarded, and it is to be understood that ferrimagnetic materials are included within the purview of the present invention. As used in this specification, the word "ferrite" is intended to include ferromagnetic materials, although it is realized that technically only ferrimagnetic materials are classed as ferrites.

Ferrites have been used extensively in microwave devices, and are assuming increasingly greater importance for use in microwave systems utilizing the microwave region of the electro-magnetic spectrum. It is well known to those skilled in the art that in crystalline ferrite structures, the magnetization tends to be directed along certain definite crystallographic axes designated as the easy axes of magnetization. The directions of these easy axes of magnetization depend upon the anisotropy constants of the material.

It has been found that some ferrite devices for use in microwave applications, such as isolators, for example, provide better operation if the easy axes of magnetization of each of the crystals which compose the material are, respectively, aligned or polarized parallel to each other. Alignment of these axes provides a material with a narrower resonance width, which usually represents an advantage in microwave system applications.

Despite the fact that it is highly desirable to obtain ferrite materials, all of whose easy axes are aligned, the materials which have heretofore been used in microwave devices have generally been composed of randomly dispersed crystals, the easy axes of magnetization of which are not aligned. This has been primarily due to the fact that up to the present time there has been no satisfactory method for producing such an orientation except in the very limited case of one dimensional alignment along only a single easy axis. In accordance with the present invention, there is provided a method and resulting structure for orienting ferrite materials, ferromagnetic materials, or ferroelectric materials, along more than one dimensional easy axis so that all the appropriate corresponding easy axes of the crystals are aligned substantially parallel to each other. As a result, a ferrite body may be produced in which all the axes of magnetization are substantially aligned.

Briefly, the present invention involves subjecting ferromagnetic or ferroelectric powders to a strong orienting field, a magnetic field in the case of ferromagnetic material and an electric field in the case of ferroelectric material. In one embodiment, the powder may be suspended in a suitable medium, for example, an epoxy resin or other suitable polymer and then subjected to the field during polymerization of the suspending medium in order to orient the crystals. The entire body of the material, ferrite powder and suspending medium, is consecutively moved through an angle which successively aligns each of the easy axes of polarization or magnetization parallel with the direction of the applied field. The time required to move through this angle should be very short compared to the time spent in the stationary positions corresponding to the easy axes' directions, so that, in effect, the material

2

is "snapped" rapidly from stationary position to stationary position. At some time during this process, the viscosity of the suspension will have increased to a value where the time required for thermal misorientation will be long compared to the positioning intervals, but not so high as to prevent orientation of the particles by the field which is being continuously applied. Upon complete solidification of the suspended medium, all of the embedded particles have a complete multi-dimensional spatial orientation in which all of the easy axes of the crystals are, respectively, aligned substantially parallel to each other.

The invention will be better understood as the following description proceeds taken in conjunction with the accompanying drawing wherein:

FIG. 1 shows the directions of the easy axes of magnetization of a cubic single crystal of ferrite material having a negative anisotropy constant;

FIG. 2 shows the directions of the easy axes of magnetization of a cubic single crystal of ferrite material having a positive anisotropy constant; and

FIG. 3 shows an exemplary system which can be utilized according to the invention for orienting ferrite material along all of its easy axes of magnetization.

25 For a material composed of cubic crystals having a negative anisotropy constant, the easy axes of magnetization lie along the four body diagonals of the cube. Such a cubic structure is shown in FIG. 1 in which the crystal is designated at 19, while the easy axes of magnetization 30 lie along the diagonals 1, 2, 3 and 4. Nickel ferrite, nickel aluminate ferrite, and manganese ferrite are examples of materials of this type.

In FIG. 2 there is shown a cubic crystalline ferrite structure which has a positive anisotropy constant. The cubic crystal 5 has its easy axes of magnetization lying along a direction parallel to the three cube edges 6, 7 and 8. Ferrites containing an appreciable amount of cobalt are examples of materials of this type.

Referring now to FIG. 3, there is shown an embodiment of the method of orienting ferrite crystal particles having a negative anisotropy constant, such as the cube shown in FIG. 1, which is accomplished by suspending the particles in a suitable viscous medium, which may be, for example, an epoxy resin such as Hysol 6020, manufactured by the Houghton Laboratories, Inc., Olean, N.Y. In the case of a ferromagnetic material, a magnetic field is continuously applied to the suspension along a direction corresponding to the direction of one of the easy axes of magnetization, the direction of field application being progressively changed in stepped movements. If the material to be oriented comprises a ferroelectric material, an electric field would be continuously applied along the direction of the respective easy axes of polarization. After the field has been applied along a first direction corresponding to a first easy axis for a sufficient time period, say on the order of ten seconds, along a first direction

say, on the order of ten seconds, along a first direction corresponding to the diagonal 1 of the body 10 shown in FIG. 1, the direction of the applied field is changed to coincide with a second direction whose geometrical relationship to the first direction corresponds to the geometrical relationship of a second body diagonal (as, for instance, body diagonal 2), and the first diagonal 1. In the case of a ferromagnetic material, the magnetic field is applied continuously for a length of time which is long compared to the time during which the test tube 20 is snapped through the angle necessary to align a next successive easy axes of polarization. For the crystal of FIG. 1, rotated about an axis normal to a crystal face, this angle would be substantially 90°. In a similar manner, the material is consecutively stepped to positions corresponding to third and fourth directions whose geometrical relationships to the first and second directions correspond

to the geometrical relationships that exist between body diagonals 3 and 4, and body diagonals 1 and 2. The continuous application of a magnetic field along each axis, together with the stepped movement from stationary position to stationary position is repeated all during the time that the viscosity of the material is increasing preferably to the point where the suspension solidifies into a solid body. The field strength used is preferably sufficient to magnetize the individual particles to saturation, i.e., as large as the anisotropy field and the saturation magnetization for the material being oriented. In the embodiment described above, the field strength may be on the order of 5,000 gauss.

If all of the particles were approximately spherical, there would be a substantially complete alignment of the crystal axes of the particles if orientation along two easy axes was obtained since the third must automatically fall in place. However, since the general shape of known particles of ferrite material is not spherical, a more perfect orientation is achieved by orienting all three easy axes, or more as the case may be, which procedure averages out the effect of shape anisotropy. The detrimental effects of a non-spherical shape of the particles can be minimized by making the time of movement through the axis angle very short. Throughout the process of continuously applying the magnetic field, the medium in which the ferrite particles are suspended is allowed to harden and, hence, its viscosity is increased. As the orientation process continues, the freedom of motion of the crystals becomes more and more restrained so that at the end of the process, the crystals are essentially "frozen" in a state such that substantially complete alignment of the respective crystal axes is attained.

The application of a continuous field along an easy axis of magnetization may be achieved in many ways, one of which is shown in FIG. 3. In this figure, a test tube 20 containing particles of a ferromagnetic material suspended within a medium 21 is positioned in the field of a coil 22 such that the direction of the magnetic field produced by a current through the coil lies along a direction corresponding to one of the body diagonals of the crystalline particles. The suspending medium may be a plastic, such as Hysol 6020, previously identified. The particles are single crystal with cubic crystal structure, and of arbitrary shape having a negative anisotropy constant. Coil 22 is arranged so that the direction of the magnetic field (as shown by the dashed arrow 26) produced by a current through the coil lies at an angle at substantially 54.4° with respect to the longitudinal direction of the test tube 20. This relationship between the longitudinal axis of the test tube and the direction of the applied field assures that, as the tube is stepped about its longitudinal axis, the field will be applied along the correct direction corresponding to the body diagonals. Coil 22 is connected to an appropriate source of excitation voltage 23.

Initially, the test tube 20 is connected to an actuating source operative to intermittently snap the test tube through the desired aligning angle by a mechanism comprising a first gear 27 attached to the test tube 20, and driven by a second gear 28 secured to the shaft 29 of a motor 35. The motor 35 is connected to a source of motor control voltage and includes appropriate mechanism for snapping the test tube through the desired solid angle. For example, well-known escapement mechanisms similar to those used in clocks and watches may be used to intermittently cause the tube 20 to be stepped. The intermittent rotation of shaft 29 causes the test tube to be moved about its longitudinal axis in the direction of the arrow 25.

During its first movement from a first stationary position to a second stationary position, test tube 20 is rotated substantially 90° from its initial position, whereupon the continuous magnetic field will be aligned with a second body diagonal axis of each of the particles in a manner similar to that in which it was aligned with the first body diagonal. Accordingly, orientation along this axis will

take place. Likewise, when the test tube 20 is stepped to positions which are 180° and 270° removed from its initial position, orientation along these axes will take place.

This process is cyclically repeated during the polymerization of the suspension 21 until the suspension has hardened. However, it is believed that substantially complete orientation is achieved before the suspension has hardened completely so that it is possible to decrease the hardening time by adding a suitable accelerator, such as Hysol Hardener C, which is manufactured and sold by the Houghton Laboratories, Inc., Olean, N.Y.

Alternatively, the suspension may be maintained in a fixed position and the coil 22 may be intermittently moved so that the field produced by it is sequentially aligned with each of the appropriate crystal axes. Any method which provides a relative motion between the suspension and the coils is suitable.

In addition, the suspension of the ferrite particles need not necessarily be limited to suspension in a plastic medium, and further need not necessarily be suspended in another material at all. As an alternative, the crystal particles may be placed in a test tube and their freedom of motion may be controlled by a pressure device, such as a piston, inserted into the test tube. The particles in the test tube may then be ultrasonically vibrated so that the particles are given substantial freedom of motion equivalent to the freedom of motion enjoyed by the particles in the plastic fluid at the start of the previously-described process. As the process continues and the test tube is moved in a stepped manner, the vibration amplitude may be gradually reduced and the pressure exerted by the piston gradually increased so that the motion of the crystal particles is gradually restrained during the process. Thus, at the end of the process, the closely-packed particles are formed into a body in which the easy axes of magnetization are correctly aligned, but in which the particles are not suspended in a plastic medium, as previously described. Alternatively, in the case of the suspended embodiment, the suspending medium may be removed, and the oriented ferrite powder sintered into a ceramic.

Although the process above-described is generally carried out at room temperature, the invention is not limited in this respect, since, in some cases, it may be desirable to perform the process at other temperatures depending upon the viscosity and rate of hardening of the plastic medium involved. In the embodiment in which Hysol was used in the plastic medium, the viscosity of the suspension at the start of the process was of the order of 50-100 poises, with substantially complete orientation being achieved when the viscosity reached a value considerably short of the substantially infinite value of viscosity which exists when the suspension is completely hardened.

Although the process of the invention has been particularly described with respect to the orientation of crystals having a negative anisotropy constant, it will be obvious to those skilled in the art that the process is also applicable to the orientation of crystals having a positive anisotropy constant. In the latter case, since the easy axes of magnetization lie along the directions of three cube edges, the application of the field will, accordingly, be in these directions. Similarly, certain hexagonal crystals having six easy axes of magnetization may also be subjected to the process of the present invention.

It can thus be seen that there has been provided multidimensionally oriented ferrite material, which may be used to advantage in transformer cores, storage elements, and magnetic amplifiers, for example. In the case of a ferrite which was oriented in only one dimension, the brittle material could not be wound in tape form so that it was impossible to realize the advantages of ferrites in this application. In accordance with the present invention, the ferrite material may now be cut into cores with the edges along the preferred axes thereby yielding the

superior characteristics obtained with tape-wound cores. In addition, the use of multi-dimensionally oriented ferrite material eliminates the microwave resonance line broadening caused by the magnetocrystalline anisotropy of randomly oriented powders.

Although there have been described what are considered to be preferred embodiments of the present invention, various adaptations and modifications thereof may be made without departing from the spirit and scope of the invention as defined in the appended claims.

What is claimed is:

1. A crystalline ferrite material comprising a plurality of minute particles suspended in a non-magnetic medium and having a plurality of crystallographic easy axes, at least one of said axes lying in a plane other than that formed by at least two other of said axes, having multi-dimensional alignment of said crystallographic easy axes formed by subjecting said material to a magnetic field, sequentially changing the direction of said magnetic field with respect to said material to align a second of said crystallographic easy axes of the particles comprising said material and gradually restraining the freedom of motion of said material while said magnetic field is being applied to solidify said material into a compact mass.

2. A ferrite body comprising a plurality of minute particles suspended in a non-magnetic medium and having a first plurality of crystallographic easy axes, at least one of said axes lying in a plane other than that formed by at least two other of said axes oriented along a second plurality of said crystallographic easy axes formed by subjecting said material to a magnetic field directed along one of said easy axes of said material, sequentially applying said field along a different crystallographic easy axis of said material and gradually restraining the freedom of motion of said material while said magnetic field is being applied to solidify the material into a compact mass.

3. A crystalline ferrite body comprising a plurality of minute particles suspended in a non-magnetic medium and having a first plurality of crystallographic easy axes, at least one of said axes lying in a plane other than that formed by at least two other of said easy axes, and having its individual particles oriented with a second plurality of said respective crystallographic easy axes in a substantially parallel alignment formed by subjecting said material to a magnetic field sequentially changing the direction of said magnetic field with respect to said material to align a second plurality of said crystallographic easy axes of the particles comprising said material and gradually restraining the freedom of motion of said material while said magnetic field is being applied to solidify the material into a compact mass.

4. A polycrystalline ferrite body comprising a plurality of minute particles suspended in a non-magnetic medium and having a first plurality of crystallographic easy axes, at least one of said axes lying in a plane other than that formed by at least two other of said axes, and having its individual particles oriented with a second plurality of said crystallographic easy axes of magnetization respectively aligned substantially parallel with each other formed by subjecting said material to a magnetic field directed along one of said easy axes of said material, sequentially applying said magnetic field along a different crystallographic easy axis of said material, and gradually restraining the freedom of motion of said material while said magnetic field is being applied to solidify said material into a compact mass.

5. The method of orienting a ferrite material having a first plurality of crystallographic easy axes, at least one of said axes lying in a plane other than that formed by at least two other of said axes, comprising subjecting said material to a magnetic field sequentially changing the direction of said field with respect to said material to align a second plurality of said crystallographic easy axes of the crystals comprising said material and gradually restraining the freedom of motion of said material while

said field is being applied to solidify said material into a compact mass.

6. The method of orienting a ferrite material having a plurality of crystallographic easy axes, at least one of said axes lying in a plane other than that formed by at least two other of said axes, said method comprising subjecting said material to a magnetic field directed along one of said easy axes of said material, sequentially applying said field along a different crystallographic easy axes of said material and gradually restraining the freedom of motion of said material while said field is being applied to solidify said material into a compact mass.

7. The method of orienting the crystals comprising a ferrite material having a first plurality of crystallographic easy axes, at least one of said axes lying in a plane other than that formed by at least two other of said axes, said method comprising suspending said crystals in a non-magnetic medium, applying a magnetic field to said suspension to align said crystals along a second plurality of said crystallographic easy axes of orientation, and gradually restraining the freedom of motion of said crystals in said suspension.

8. The method of orienting the crystals comprising a ferrite material having a first plurality of crystallographic easy axes, at least one of said axes lying in a plane other than that formed by at least two other of said axes, said method comprising suspending said crystals in a non-magnetic medium, and sequentially applying a continuous magnetic field to said suspension to align said crystals along a second plurality of said crystallographic easy axes of magnetization while gradually restraining the freedom of motion of said crystals in said suspension.

9. The method of orienting ferromagnetic crystals having a first plurality of crystallographic easy axes, at least one of said axes lying in a plane other than that formed by at least two other of said axes, said method comprising applying a magnetic field to said crystals, and sequentially moving said crystals with respect to the direction of said magnetic field to align said crystals with a second plurality of said crystallographic easy axes of magnetization substantially parallel with each other while causing said crystals to compact into a solid mass.

10. The method of orienting the crystals of a ferrite body having a first plurality of crystallographic easy axes, at least one of said axes lying in a plane other than that formed by at least two other of said axes, said method comprising suspending said crystals in a plastic non-magnetic medium that initially provides freedom of motion for said crystals, subjecting said suspension to a continuous magnetic field, and relatively moving said suspension with respect to said field in order to polarize said crystals along a second plurality of said crystallographic easy axes of magnetization while progressively restraining the freedom of motion of said crystals to form a compact body.

11. The method of orienting a body of ferromagnetic material having a plurality of crystallographic easy axes, at least one of said axes lying in a plane other than that formed by at least two other of said axes, said method comprising suspending said crystals in a plastic non-magnetic medium, and applying a continuous magnetic field to said medium while said medium is snapped to different positions in said field, and causing said plastic medium to gradually harden.

12. The method of orienting a ferrite body composed of substantially cubic crystals wherein the crystallographic easy axes of magnetization correspond to the body diagonals of said crystals, said method comprising suspending said crystals in a plastic non-magnetic medium, subjecting said suspension in a first position to a continuous magnetic field to align said crystals along one of said easy axes, moving said suspension to a different crystallographic easy axis position in said field during a time interval which is short compared to the time interval spent in said first position while gradually causing said suspension to harden.

13. The method of orienting the crystals comprising a ferrite material having a first plurality of crystallographic easy axes, at least one of said axes lying in a plane other than that formed by at least two other of said axes, said method comprising suspending said crystals in a non-magnetic medium, applying a continuous magnetic field to said suspension to align said crystals along a second plurality of said crystallographic easy axes of magnetization while gradually restraining the freedom of motion of said crystals in said suspension, and heating said suspension to remove said medium, whereby said crystals are sintered into a ceramic mass.

14. The method of orienting the ferromagnetic crystals having a first plurality of crystallographic easy axes, at least one of said axes lying in a plane other than that formed by at least two other of said axes, said method comprising suspending said crystals in a non-magnetic medium, applying a continuous magnetic field to said suspension to align said crystals along a second plurality of said crystallographic easy axes of magnetization while gradually restraining the freedom of motion of said crystals in said suspension, and heating said suspension to remove said medium, whereby said crystals are sintered into a ceramic mass.

## References Cited in the file of this patent

## UNITED STATES PATENTS

|    |           |                     |                |
|----|-----------|---------------------|----------------|
| 5  | 2,532,876 | Asche et al. -----  | Dec. 5, 1950   |
|    | 2,687,500 | Jones et al. -----  | Aug. 24, 1954  |
|    | 2,762,778 | Gorter et al. ----- | Sept. 11, 1956 |
|    | 2,827,437 | Rathenau -----      | Mar. 18, 1958  |
|    | 2,837,483 | Hakker et al. ----- | June 3, 1958   |
| 10 | 2,964,793 | Blume -----         | Dec. 20, 1960  |
|    | 2,974,104 | Paine et al. -----  | Mar. 7, 1961   |

## FOREIGN PATENTS

|         |                     |              |
|---------|---------------------|--------------|
| 758,320 | Great Britain ----- | Oct. 3, 1956 |
|---------|---------------------|--------------|

## OTHER REFERENCES

Morrill: General Electric Review, August 1950, pp. 16-21.

Stuijts et al.: Philips Technical Review, vol. 19, 1957/58, No. 7-8, pub. Feb. 10, 1958, pp. 209-217.

Watson et al.: Journal of Applied Physics, vol. 29, No. 3, pp. 306-308, March 1958.

Popper: Journal of Electrical Engineers, vol. 2 (new series), No. 20, pp 450-457.